

# UNITED STATES PATENT OFFICE.

LAYTON M. PARKHURST, OF CHICAGO, ILLINOIS, ASSIGNOR, BY MESNE ASSIGNMENTS, TO H. KRAMER & CO., OF CHICAGO, ILLINOIS, A CORPORATION OF ILLINOIS.

## ANTIFRICTION ALLOY AND METHOD OF MANUFACTURE.

1,359,194.

Specification of Letters Patent. Patented Nov. 16, 1920.

No Drawing.

Application filed March 8, 1920. Serial No. 364,035.

To all whom it may concern:

Be it known that I, LAYTON M. PARKHURST, a citizen of the United States, and a resident of the city of Chicago, in the county of Cook and State of Illinois, have invented certain new and useful Improvements in Antifriction Alloys and Methods of Manufacture; and I do hereby declare that the following is a full, clear, and exact 10 description of the same.

This invention relates to anti-friction alloys and method of manufacture.

Anti-friction alloys should possess three properties; low coefficient of friction, sufficient hardness to withstand bearing pressure, and resistance to heat not only as regards fusibility but also oxidation, crystallization, and segregation of constituents under heat.

20 Lead possesses a very low coefficient of friction but is not hard enough to stand even moderate bearing pressures. Even Babbitt metal cannot be used with bearing pressures over 100 lbs. per square inch.

25 Further, lead and antimony have the property of combining with each other in all proportions without impairing the anti-friction properties of either. The antimony hardens the lead, and when mixed in the proportion 30 of 80 parts of lead by weight with 20 parts of antimony possesses greater antifriction or wearing properties, or will stand a higher speed without heat or abrasion than any other proportions of these two metals. Such

35 an alloy is not, however, sufficiently hard for automobile truck bearings or the like which have high bearing pressures around 600 to 700 lbs. per square inch. Further, such an alloy is not resistant to heat and its 40 use, therefore, is usually restricted to light high-speed machinery.

None of these antifriction alloys, including those sold under the name of Babbitt metal, has a hardness of over 22 or 23 on 45 Dr. Brinnell's scale.

One of the objects of the present invention is to provide an antifriction alloy capable of being used successfully with shaft pressures up to and even exceeding 1,000 lbs. 50 per square inch.

A further object is to provide an antifriction alloy which is resistant to the action of heat.

It is also an object of the invention to provide a method of making an antifriction

alloy without the use of temperatures in excess of about 350°—C.

In general it is an object of this invention to provide an improved antifriction alloy and method of manufacturing the same.

I have found that the hardness of a lead-antimony alloy may be increased by replacing a part of the antimony by tin and copper. I have also discovered that greatly improved results are obtained by alloying the 65 tin and copper at a temperature below that at which copper melts. A further discovery I have made is that small additions of certain substances, notably phosphorus, increases the hardness very materially.

An antifriction alloy adapted for use with bearing pressures up to 1,000 lbs. per square inch may be made as follows:

|            |     |    |
|------------|-----|----|
| Lead       | 79% | 75 |
| Antimony   | 12% |    |
| Tin        | 6%  |    |
| Copper     | 2.5 |    |
| Phosphorus | 0.5 |    |

If the bearing pressure is greater than 80 1,000 lbs. per square inch the proportion of copper to antimony may be increased to advantage in order to make the product harder. The above alloy, made by alloying the copper with the tin at a low temperature and then mixing the product with antimony, phosphorus and lead, has a hardness of 27.5 to 28.0. Without the phosphorus the hardness is about 26.0 to 26.5.

The proportions of the various constituents may be varied considerably without reducing the hardness, heat-resisting, and other properties beyond useful limits. Ordinarily, however, the proportions should be retained within the following limits:

|            |      |       |     |
|------------|------|-------|-----|
| Lead       | 73%  | — 85% | 90  |
| Antimony   | 8    | — 14  |     |
| Tin        | 5    | — 7   |     |
| Copper     | 1.5  | — 3.5 | 85  |
| Phosphorus | 0.25 | 0.7   | 100 |

It has been found in particular that usually additions of phosphorus above 0.7% tend to soften instead of harden the product.

The melting points of the various constituent metals are as follows: lead 327°—C.; antimony, 630°—C.; tin, 232°—C.; and copper, 1083°—C. By adding the constituents in proper sequence the temperature of the melt may be retained below 350°—C. at all 110

times. In the first place the tin is melted and the copper added thereto, maintaining the temperature preferably not in excess of 300°. When the copper has completely dissolved in the tin and a true homogeneous alloy produced the necessary amount of antimony and phosphorus is added. This may, if desired, be cast into blocks for incorporation with batches of lead at a later date.

10 The lead is melted and the requisite amount of the above alloy added thereto to give a metal having the desired composition. In some cases the antimony may be added to the lead instead of to the tin-copper alloy

15 since antimony readily alloys with lead in all proportions.

One of the great advantages of keeping the temperature of the tin-copper alloy below 300°—C. is avoidance of oxidation. Such alloys not only readily oxidize but also dissolve oxygen which is given off again on cooling. Such oxidation and (or) solution of oxygen as may take place at 300°—C. is counteracted by the phosphorus added which 25 combines with the oxygen yielding a homogeneous, dense, and strong product. The phosphorus, therefore, has two functions: first, to increase the hardness, and second, to de-oxidize the alloy.

30 While I have described my invention in a preferred form, I am aware that changes and modifications may be made in the in-

gredients employed and the proportions and manner in which they are mixed without departing from the principles of my invention, and I do not, therefore, purpose limiting the patent granted otherwise than necessitated by the prior art.

I claim as my invention:

1. An antifriction alloy comprising approximately 79% lead, 12% antimony, 6% tin, 2.5% copper and 0.5% phosphorus.

2. An antifriction alloy comprising approximately 73%—85% lead, 8%—14% antimony, 5%—7% tin, and 0.25%—0.70% phosphorus.

3. The method of making an antifriction alloy comprising alloying copper and tin, adding thereto antimony and phosphorus, and finally mixing the product with lead.

4. The method of making an antifriction alloy comprising melting tin and alloying a smaller proportion of copper therewith at a temperature not substantially in excess of 300°—C., adding thereto antimony and phosphorus and finally mixing the product with molten lead.

In testimony whereof I have hereunto subscribed my name in the presence of two subscribing witnesses.

LAYTON M. PARKHURST.

Witnesses:

RIDSDALE ELLIS,  
EARL M. HARDINE.